

Feb. 3, 1948.

M. S. HUDSON

2,435,219

ART OF DEHYDRATING AND IMPREGNATING WOOD

Filed Sept. 17, 1947



*Inventor*

MONIE S. HUDSON

*By Parrott and Richards  
Attorneys*

## UNITED STATES PATENT OFFICE

2,435,219

ART OF DEHYDRATING AND IMPREG-  
NATING WOOD

Monie S. Hudson, Spartanburg, S. C.

Application September 17, 1947, Serial No. 774,639

7 Claims. (Cl. 117—57)

1

This application is a continuation-in-part of my copending application Ser. No. 324,893, filed March 19, 1940, now U. S. Patent No. 2,273,039, granted February 17, 1942, and my copending application Ser. No. 431,176, filed February 16, 1942, and allowed April 4, 1947.

In my above Patent 2,273,039 I have disclosed and claimed a process for drying wood with heated organic vapors, the process being carried out in a closed chamber in which the atmosphere is substantially saturated with organic vapor; that is, as rapidly as the moisture is liberated from the wood during the drying process it is removed from the chamber so that the atmosphere around the wood is substantially saturated with organic vapor. The temperature in the drying chamber is maintained above 212° F. and up to about 450° F. That method of drying wood with an atmosphere composed substantially entirely of the organic medium enabled wood and wood products to be dried commercially in a matter of hours instead of days as was required in prior conventional practice. One practical objection to that process is the relatively high cost of the fuel for vaporizing the organic compounds and the cost of handling the relatively large amount of organic vapor condensate produced during the drying operation. This is especially true where concentrations of about 99%-100% organic vapor are attempted to be maintained.

In accordance with the present invention, I have discovered that a substantially saturated atmosphere of organic vapor in the drying chamber, as disclosed in my above patent, is not necessary and that, within certain limits, moisture vapor may be permitted in the drying chamber, and with substantially less fuel and handling costs. An important factor is to prevent too long a drying time which would cause hydrolysis of the wood in the presence of the moisture vapor and would also involve excessive costs of operation of the drying cylinder for such long period of time.

I have found that the extreme limit of water vapor is around 50% (the other 50% being organic vapor) and that operation at or above that percentage of water vapor is unreliable and protracts the drying operation much too long; and that a good reliable and economical percentage of water vapor is approximately 35%. At this percentage the organic vapor content of the atmosphere in the drying chamber would be approximately 65%.

This organic vapor percentage may be increased (with corresponding decrease in the water vapor content) up to 100%, theoretically, but I have found from actual experience in the commercial operation of the process that there is no real practical advantage in increasing the organic vapor content above about 90%; and that

2

a good commercially advantageous range is about 65% to 90% organic vapor, with a corresponding moisture vapor range of about 35% to 10%. The higher the percentage of organic vapor the faster the drying time but within the above commercial operating range of approximately 65% to 90% the drying time does not vary greatly and the operation is stable and reliable over this range. This is illustrated by the flat portion of the curve as shown in the accompanying drawing in which:

The single figure in the drawing is a graphic illustration of the relationship between the drying atmosphere concentration and varying time, characteristic of the drying process of this invention.

The curve shown in the drawing is based upon data from various tests that I have made but is to be understood as representative only generally of the relationship between % drying vapor concentration and hours drying time for my process. It would naturally vary some with each particular type and size of timber or other wood products being dried. The very steep part of the curve corresponding to about 50% and less of organic vapor shows that a slight decrease in percentage of organic vapor causes a very large increase in the drying time. Accordingly it is not practical to operate under conditions that fall under that portion of the curve.

At the other extreme limit, that is, approximately 100% organic vapor, the curve is flat and from the standpoint of time of operation, it is satisfactory, in fact, it is optimum. However, practical experience has shown that the cost of operation rises extremely rapidly as a saturated organic vapor atmosphere is approached and that above 99% organic vapor the cost goes infinitely high.

It is therefore apparent from the above facts and from the curve in the drawing that the range of about 65% to 90% is a good, safe, and commercially advantageous range in which to operate, and that the organic vapor percentage may be increased or decreased to some extent on either side of this range but without any great benefit. As compared with the saturated atmosphere process of my above patent, the process of the present application, especially when operated in the approximate 65% to 90% range, results in a very substantial reduction in the fuel cost, for heating the organic medium, and a substantial reduction in the amount of organic condensate which must be handled and reclaimed during the drying operation.

In carrying out the process of my invention I use any suitable drying apparatus having a closed chamber and which is preferably maintained at substantially atmospheric pressure, although in some cases a reduced pressure or vacuum may be employed. An example of a suita-

ble apparatus is illustrated and described in detail in my copending application Ser. No. 431,177, which was filed concurrently with my above identified application Ser. No. 431,176, of which the present application is a continuation-in-part; the said application Ser. No. 431,177 having been allowed on May 7, 1947. For the operation of my process with that equipment, vapor-pressure-temperature relations of the organic material to be used in the process are determined on samples, and a graph made up by using Dalton's law calculations showing the relation of percentage of weight of organic material in the vapor phase, (water being the "B" component) to temperature. A temperature corresponding to a concentration of about 65%, for example, of organic material in the vapor phase is selected from this chart. This temperature is then set on a thermostatic-recording controller whose actuating bulb is situated in the drying chamber of the drying apparatus.

This controlling device operates a suitable mechanism for varying the heat input to the evaporator which might be part of or a separate vessel from the drying chamber. In this evaporator, the organic drying medium is maintained at its boiling point, and any impulse set up by the thermostatic controller increases or decreases the heat input, which modifies the boil-up of organic drying material into the cylinder, thus maintaining the concentration of organic material always within the desired critical limit.

The wood or wood products to be dried are placed in the drying chamber, and the temperature used is one which will assure in the apparatus throughout the actual drying period (exclusive of the short start-up period), an organic vapor concentration within the range of approximately 65% to 90%. To insure an accurate check on this, during drying, I employ suitable meters and a continuously separating device by which the proportion of organic material to water in the condensate may be measured and held at the desired percentage by controlling the heat input to the system.

Suitable organic drying media for use in the present invention are listed below, and some of these are also excellent preserving materials for wood and wood products. Furthermore, where impregnation with preservative drying media is desired, this may be accomplished substantially with the drying, so that drying and preserving is carried out as a single step, thus eliminating the subsequent pressure impregnation cycle which is necessary if a non-preserving drying agent is used.

Preferred examples of suitable organic drying media are:

- (1) Distillates of petroleum and coal tar and distillates of wood and wood tar.
- (2) Alcohols, such as butyl, isobutyl, amyl, diethylene glycol, or glycerol.
- (3) Aldehydes, such as butyric or furfural.
- (4) Amines, such as aniline or quinoline.
- (5) Esters, such as glycol mono-ethyl-ether acetate or butyl—or amylacetates.
- (6) Ethers, such as diethyl ether.
- (7) Halides, such as dichloro phenol, tetrachlorophenol, pentachlorophenol and para-dichlorobenzene.
- (8) Nitro compounds, such as nitrobenzene or orthonitro-chlorobenzene.
- (9) Hydrocarbons, such as mesitylene, xylene, toluene, benzene, dipentene, or diphenyl.
- (10) Phenols, creosols, or xylenols.

For simultaneous drying and impregnating, numerous of the above compounds or mixtures thereof are satisfactory, e. g., tetrachlorophenol alone or in solution in a petroleum distillate. Compounds having boiling points at temperatures higher than can be used in contact with the wood may be utilized in solution in solvents that abnormally raise their vapor pressures so that they can be distilled at lower temperatures.

Certain of the high melting point compounds will be found to possess vapor pressures that are too low for satisfactory operation as drying and impregnating media at atmospheric pressure, that is, too high a temperature would be required to volatilize appreciable amounts at atmospheric pressure even though a solvent which raises the vapor pressure of the solute abnormally, is used. This difficulty may be easily overcome by employing a liquid solvent having a boiling point near that of the toxic solute and impressing vacuum on the system to lower the boiling point of the mixture.

The term "wood and wood products" as used herein is intended to comprehend such materials as green or partially seasoned poles, pilings, cross-ties, structural timbers, boards and other lumber, plywood, shavings, wood chips in various forms, pulps, wood flour of various kinds, wood molding powders, etc.

I claim:

1. A rapid, high temperature method of dehydrating wood in a closed space, which is characterized by commercial drying of the wood in a matter of hours instead of days, comprising subjecting the wood to a highly heated vapor composition containing not substantially less than about 65% by weight of an inert organic vapor but less than a saturated atmosphere of said vapor, and an appreciable amount of water vapor not in excess of about 35% by weight, said organic vapor being of a type suitable for permeating the wood and replacing the water in said wood and having no adverse effects on the wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% by weight at any time during the drying treatment, and continuing this treatment until the desired degree of dryness of the wood is obtained.
2. A rapid, high temperature method of dehydrating wood in a closed space, which is characterized by commercial drying of the wood in a matter of hours instead of days, comprising subjecting the wood to a highly heated vapor composition containing approximately 65% to 90% by weight of an inert organic drying vapor and approximately 10% to 35% by weight of water vapor, said organic vapor being of a type suitable for permeating the wood and replacing the water in said wood and having no adverse effects on the wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% at any time during the drying treatment, and continuing this treatment until the

desired degree of dryness of the wood is obtained.

3. A rapid, high temperature method of dehydrating wood in a closed space, which is characterized by commercial drying of the wood in a matter of hours instead of days, comprising subjecting the wood to a highly heated vapor composition maintained at a temperature substantially within the range of about 212° F. to 450° F. and containing not substantially less than about 65% by weight of an inert organic vapor but less than a saturated atmosphere of said vapor, and an appreciable amount of water vapor not in excess of about 35% by weight, said organic vapor being of a type suitable for permeating the wood and replacing the water in said wood and having no adverse effects on the wood, and said vapor composition being heated to and maintained during drying at a temperature substantially above the vaporization temperature of the moisture in the wood so that the moisture is flashed off as vapor, progressively displacing the liberated moisture vapor so that the water vapor content of said drying vapor composition does not substantially exceed 35% at any time during the drying treatment, and continuing this treatment until the desired degree of dryness of the wood is obtained.

4. A rapid, high temperature method of dehydrating wood in a closed space, which is characterized by commercial drying of the wood in a matter of hours instead of days, comprising subjecting the wood to a highly heated vapor composition containing not substantially less than about 65% by weight of an inert vapor of a wood preservative organic compound but less than a saturated atmosphere of said vapor, and an appreciable amount of water vapor not in excess of about 35% by weight, said organic vapor being of a type suitable for permeating the wood and replacing the water in said wood and having no adverse effects on the wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% at any time during the drying treatment, and continuing this treatment until the desired degree of dryness of the wood is obtained and the wood is impregnated after the drying treatment with said wood preservative organic compound.

5. A rapid, high temperature method of dehydrating wood in a closed space, which is characterized by commercial drying of the wood in a matter of hours instead of days, comprising, maintaining a reduced pressure in said closed space, subjecting the wood to a highly heated vapor composition containing not substantially less than about 65% by weight of an inert organic vapor but less than a saturated atmosphere of said vapor, and an appreciable amount of water vapor not in excess of about 35% by weight, said organic vapor being of a type suitable for permeating the wood and replacing the water in said wood and having no adverse effects on the

wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% by weight at any time during the drying treatment, and continuing this treatment until the desired degree of dryness of the wood is obtained.

6. A rapid, high temperature method of dehydrating wood in a closed space, which is characterized by commercial drying of the wood in a matter of hours instead of days, comprising subjecting the wood to a highly heated vapor composition containing not substantially less than about 65% by weight of an inert organic vapor but less than a saturated atmosphere of said vapor, and an appreciable amount of water vapor not in excess of about 35% by weight, said organic vapor containing a toxic preservative compound, and being of a type suitable for permeating the wood and replacing the water in said wood and having no adverse effects on the wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% by weight at any time during the drying treatment, and continuing this treatment until the desired degree of dryness of the wood is obtained.

7. A rapid, high temperature method of dehydrating wood in a closed space, which is characterized by commercial drying of the wood in a matter of hours instead of days, comprising subjecting the wood to a highly heated vapor composition containing not substantially less than about 65% by weight of an inert organic vapor but less than a saturated atmosphere of said vapor, and an appreciable amount of water vapor not in excess of about 35% by weight, said organic vapor being obtained by heating an organic compound selected from the group consisting of distillates of petroleum, coal tar, wood and wood tar, the said organic vapor being of a type suitable for permeating the wood and replacing the water in said wood and having no adverse effects on the wood, and said vapor composition being heated to and maintained during drying at a high temperature substantially above the vaporization temperature of the moisture in the wood so that the moisture is flashed off as vapor, progressively displacing the liberated moisture vapor so that the water vapor content of said drying vapor composition does not substantially exceed 35% by weight at any time during the drying treatment, and continuing this treatment until the desired degree of dryness of the wood is obtained.

MONIE S. HUDSON.

**Certificate of Correction**

Patent No. 2,435,219.

February 3, 1948.

**MONIE S. HUDSON**

It is hereby certified that error appears in the printed specification of the above numbered patent requiring correction as follows: Column 3, line 51, for the word "substantially" read *simultaneously*; and that the said Letters Patent should be read with this correction therein that the same may conform to the record of the case in the Patent Office.

Signed and sealed this 6th day of April, A. D. 1948.

[SEAL]

**THOMAS F. MURPHY,**  
*Assistant Commissioner of Patents.*